

# United States Patent Office

3,316,122

Patented Apr. 25, 1967

1

3,316,122

## PROCESS OF BONDING NONWOVEN FABRIC WITH CHLORINATED ATACTIC POLYPROPYLENE AND THE BONDED FABRIC

Walter B. Armour, Plainfield, N.J., Gerald H. Brown, Syracuse, N.Y., and Emil D. Mazzarella, Plainfield, N.J., assignors to National Starch and Chemical Corporation, New York, N.Y., a corporation of Delaware  
No Drawing. Filed Feb. 20, 1964, Ser. No. 346,092  
8 Claims. (Cl. 117—136)

This invention relates to novel binding compositions for use in the preparation of nonwoven fabrics. More particularly, it relates to the preparation of nonwoven fabrics which are characterized by their excellent fire retardancy as well as by their unusual degree of softness and strength.

Nonwoven fabrics are fabrics which are neither woven, knitted, spun nor made by conventional wool felting processes. They are, instead, built up through the interlocking of fibers by means of chemical bonding agents or fusible fibers. This is accomplished by any combination of mechanical means, chemical action, or heat. Nonwoven fabrics may thus be broadly defined as a textile structure consisting of a web or mat of fibers held together with a binding material.

In preparing these nonwoven fabrics it is possible to use either natural or synthetic fibers. Thus, among the fibers which may be used in nonwoven fabrics are cotton, rayon, cellulose acetate, and triacetate, nylon, acrylic, polyester, glass, vinyl polymer and copolymer fibers, as well as paper fibers, wood pulp fibers, and fibers derived from waste paper. Generally, different types of fibers are blended in order to achieve the desired end product properties. After being blended, the individual fibers are then picked or shredded so as to obtain a more uniform distribution. These initial operations serve to prepare the fibers for the web forming process which employs various complex web forming machines. These machines produce a web or flimsy sheet of fibers which will not remain in one piece by itself, but has to be supported by conveyors.

At this point in the process, the web must be bonded and this may be accomplished by mechanical means which entangle the fibers and thus give strength to the web. However, binding is more usually accomplished by the use of a chemical binding agent which may be in the form of an emulsion, a powder, a solvent, or a solution. These binding agents can be applied to the nonwoven web by immersion, spraying, in the form of a foam, by rolls or pads, or by the sprinkling of dry thermoplastic resins. The web can be completely covered with the binding agent or the binding agent may be applied so as to form a discontinuous pattern by processes similar to printing. Thermoplastic fibers may also be used to accomplish binding by being blended into the fiber mixture or by using them as the sole component of the web. Application of heat causes these fibers to become tacky and thus stick to each other and/or to other non-thermoplastic fibers.

The formation of a nonwoven gauze differs, in some respects, from the preparation of a nonwoven fabric. Rather than being formed into a web, the fibers are, instead, made into yarns which are aligned parallel to each other. These yarns, which represent the warp yarns of the gauze, are then run through a saturation bath wherein a series of steel cones mechanically meter the amount of binding agent that is applied to the warp yarns. The wet warp yarns are thereupon adhered to a series of fill yarns which comprise parallel aligned yarns positioned perpendicularly with respect to the wet warp yarns. The complete gauze is then dried by any suitable means such as

2

by being passed over a drying drum or a heated calendar stack.

Various materials have been employed as binding agents for nonwoven fabric and gauze, including such binders as polyvinyl acetate, polyacrylates, polyvinyl chloride, urea-formaldehyde resins, and the like. None of these binding agents, however, have been entirely satisfactory, primarily because of prohibitive costs and/or unsatisfactory properties imparted to the resulting nonwoven products.

Thus, for example, it is well known that many of the binding agents heretofore utilized have provided nonwoven fabrics with very little, if any, resistance to fire and flame propagation and, in some cases, these binders have even served to increase the flammability of the fabric. Fire resistance is, of course, of great importance in nonwoven fabrics which are to be used in either consumer or industrial applications wherein they may tend to become accidentally ignited. Unfortunately, in attempting to provide binders which successfully imparted fire retardancy, it was found that the binders which were desirable in this respect were often deficient with regard to their adhesive and/or processing characteristics.

In addition to the above described fire retardancy problem, water resistance, tensile strength, edge tear, and elongation of nonwoven products have often proved deficient when binders heretofore known have been utilized. Moreover, since nonwoven fabrics are widely used in wearing apparel, upholstery, floor and wall coverings, and similar applications, it is often desirable that such fabrics possess a degree of softness, or, as it is commonly referred to, a good "hand" or feel. This latter property has often lacking in nonwoven products when the binding agents of the prior art have been used in their manufacture.

Thus, it is an object of this invention to provide binding compositions for nonwoven fabrics and gauze, the use of which results in nonwoven materials which are characterized by their outstanding resistance to fire and flame propagation as well as by their desirable characteristics of wear and feel. Other objects and advantages of this invention will be apparent from the discussion which follows hereinafter.

We have now discovered that the use of chlorinated atactic polypropylene as a binder for nonwoven fabrics provides the resulting products with outstanding fire retardancy properties. In addition, the use of this novel binder imparts highly desirable properties of water resistance, tensile strength, edge tear, and elongation to said fabrics and also provides them with a remarkable degree of softness. Moreover, the latter characteristic of softness of "hand" is realized without any sacrifice in the strength of the resulting nonwoven products.

In accordance with the invention, nonwoven products are prepared by means of a process involving the application, to a nonwoven sheet or web of fibers, of a binder composition comprising chlorinated atactic polypropylene which may be in the form of either a lacquer or an aqueous emulsion.

Polypropylene is a synthetic resin which, of late, has enjoyed greatly increased usage in the preparation of molded articles, fibers and films. For use in the late applications it is desirable that the polypropylene should have a highly crystalline structure which thereby serves to increase the strength of this versatile plastic. The inherent crystallinity of polypropylene, is in turn, dependent upon its molecular structure or configuration. Thus, crystalline propypropylene molecules will exhibit a so-called isotactic structure wherein the methyl groups will be regularly distributed on the same side of the polymer

chain in a manner analogous to that shown in the following diagram:



On the other hand, polypropylene which is not crystalline will exhibit a so-called atactic structure wherein the methyl groups are randomly distributed on either side of the polymer chain in a manner analogous to that shown in the following diagram.



In manufacturing polypropylene, the processes currently employed make use of so-called stereospecific catalysts which are chosen for their ability to provide the resulting polypropylene with an isotactic structure and thereby impart a maximum degree of crystallinity to the polymer. However, despite the use of these catalysts, present polymerization techniques still produce a product with a significant proportion of atactic polypropylene. The presence of this non-crystalline fraction would, of course, detract from the strength of any articles manufactured from such polypropylene. Therefore, it is the practice in the art to separate this atactic portion from the crystalline material and this is readily accomplished by means of a solvent extraction technique. To date, very few, if any, applications have been found for this atactic polypropylene residue. Its inherent lack of crystallinity obviates its use in the preparation of films, fibers, and molded products; while any use of this material as an adhesive base is similarly precluded since the resulting adhesive films are exceedingly soft and display relatively little strength.

The chlorinated atactic polypropylene which is used as the binding agent in the process of our invention is prepared by dissolving the atactic polypropylene in a non-reactive organic solvent such as carbon tetrachloride, methylene chloride, chlorobenzene, or chloroform. The atactic polypropylene is then chlorinated in the presence of a suitable catalyst which may be a solvent soluble organic peroxide, such as benzoyl peroxide or lauroyl peroxide, or a metal salt, such as ferric chloride or aluminum chloride. The latter catalysts are usually present in the reaction mixture in a concentration of about 0.1 to 1.0%, by weight, of the atactic polypropylene undergoing chlorination. Chlorination may be accomplished by bubbling chlorine gas directly onto the reaction mixture or by refluxing the latter in the presence of a chlorination agent such, for example, as sulfuryl chloride or thionyl chloride.

For use as a binding agent in the process of our invention, the chlorinated atactic polypropylene may contain from about 8 to about 35%, by weight, of chlorine.

A typical procedure, in this case employing sulfuryl chloride, which may be utilized for the chlorination of atactic polypropylene would involve first preparing an organic solvent solution of the atactic polypropylene with the process of solution being assisted by subjecting the mixture to mechanical agitation as well as by heating it to reflux. While the thus prepared solution is maintained under reflux and agitation, the selected catalyst is

introduced therein. The sulfuryl chloride is then slowly added with the solution being maintained at reflux for a

period which may range from about 5 to 10 hours, thereby yielding the desired chlorinated atactic polypropylene. It may be noted that the above described chlorination procedure may also be utilized with thionyl chloride. However, when gaseous chlorine is used, this procedure

is modified somewhat in that the reaction temperatures are maintained below reflux levels.

In using chlorinated atactic polypropylene as the binding agent in the manufacture of nonwoven fabrics, there are several possible techniques for their application to the fiber web. These include saturation bonding, wet-roll bonding, spray bonding, and segmental bonding. Saturation bonding, which is also referred to as continuous, immersion, solution or impregnation bonding, is the most commonly used bonding method and consists simply of passing the fragile fiber web through a liquid binder bath. The web is then passed through squeeze rolls to remove the excess binding agent. Wet-roll bonding is similar to the saturation process, the main difference being that the web does not go through the liquid bath. Instead, a series of mechanical rolls pick up the binder and transfer it to the moving web. Spray bonding applies the liquid binding agent by spraying a fine mist of binder over the surface of the web. And, segmental bonding, which is also referred to as discontinuous, patterned, print, engraved, intermittent, and spot bonding, is the process wherein the binding agent is applied to the web in a uniform pattern, resulting in definite bonded and unbonded portions upon the web surface.

With the above described application techniques, or with any other procedures which may be devised by the practitioner, it is desirable that the finished nonwoven fabric or gauze contain from about 3% to 280% of binding agent, i.e., chlorinated atactic polypropylene solids, as based on the weight of the dry fibers in the finished nonwoven product. Particularly effective fabrics were obtained wherein the finished product contained from about 50% to 200% of binding agent. The desired binder content can be realized by proper adjustment of the solids content of the binding agent lacquer or emulsion and/or by varying by means well known to those skilled in the art, the initial pickup by the fiber web or warp yarns of the binding agent.

Subsequent to the application of our chlorinated atactic polypropylene binding agent, the sheet or web of nonwoven fabric may be dried at room or elevated temperatures. The drying cycles used in this process depend upon the temperature employed, the rate and amount of air flow, and other factors inherent in the practitioner's facilities and method of operation. In any case, temperatures varying from room temperature to about 350° F. may be used to remove the solvent or water that is present in the wet web.

When the binders of our invention are utilized in the

form of laquers, it is possible to use various solvents in their preparation. Thus, for example, chlorinated atactic polypropylene may be dissolved in a variety of solvents, including: aromatic hydrocarbons, such as toluene and xylene; cyclic hydrocarbons, such as decahydronaphthalene and tetrahydronaphthalene; aliphatic hydrocarbons containing from 5 to 11 carbon atoms, such as pentane, hexane, and nonane; and, chlorinated hydrocarbons, such as methylene chloride, carbon tetrachloride, tetrachloroethylene, perchloroethylene, and also chlorinated aromatic hydrocarbons such as chlorobenzene. It should be noted that, where so desired by the practitioner, it is possible to prepare these lacquers with various combinations of any of the above listed solvents. The resin solids content of these chlorinated atactic polypropylene lacquers should usually range from about 1% to about 50% by weight.

When the chlorinated atactic polypropylene is employed in our invention in the form of an aqueous emulsion, the latter may be prepared by adding an aqueous solution of an emulsifying agent, such as polyvinyl alcohol, morpholine-oleic acid mixtures, and the like, to an organic solvent solution of chlorinated atactic polypropylene; the latter solution having been prepared by the use of any of the above listed solvents. Water is then added with vigorous agitation, the amount of water added depending upon the solids content desired in the ultimate emulsion. In those cases where the organic solvent has a boiling point less than that of water, it can be removed from the emulsion by distillation or other appropriate means. The resin solids content of these chlorinated atactic polypropylene emulsions usually ranges from about 2 to 65%, by weight.

It should be mentioned that various additives, such as defoamers, lubricants, antioxidants, and the like, may be added to our chlorinated atactic polypropylene binder formulations in order to enhance the properties imparted to the nonwoven fabrics to which said binders are applied. It may also be noted that our chlorinated atactic polypropylene binders may be used in combination with various thermosetting and thermoplastic resin binders.

In the following examples, which further illustrate the embodiment of our invention, all parts given are by weight unless otherwise indicated.

#### Example I

This example illustrates the preparation of fire retardant nonwoven fabrics using lacquers and emulsions of chlorinated atactic polypropylene as the binding agents therefor.

In this example, and in the examples that follow, the same basic procedure was utilized in preparing the nonwoven fabric. In this basic procedure, a web was bonded as it passed through the nip of a padder, the binding agent being applied by a stainless steel transfer roll which dipped into a pan containing the binding agent and transferred the impregnant to the passing web. The amount of binding agent picked up by the web was determined by the pressure at the nip as well as by the initial solids content of the binding agent. The wet web was then passed into a forced draft oven and dried at 300° F. for a period of 3 minutes. This drying operation effected a complete removal of water or solvent and the web was thereupon cooled to room temperature.

(a) 4 parts of oleic acid and 4 parts of morpholine were added to 100 parts of a 40% hexane solution of chlorinated atactic polypropylene having a chlorine content of 10%, by weight. 85 parts of water were then added with vigorous agitation. The hexane was removed from the emulsion by distillation, and the solvent-free emulsion was diluted with water to a final concentration of 1%, by weight, of chlorinated atactic polypropylene solids. A nonwoven sheet composed of 95/5 rayon/cellulose fibers was passed through this emulsion, squeezed between rollers, and dried at room temperature. In this

case, the nip pressure was adjusted so as to yield a finished fabric containing 3%, by weight, of chlorinated atactic polypropylene solids, as based on the dry fiber weight.

5 (b) A nonwoven sheet composed of 95/5 rayon/cellulose fibers was passed through a 2%, by weight, hexane lacquer of chlorinated atactic polypropylene having a chlorine content of 30%, by weight. The sheet was thereafter squeezed between rollers, and dried at room temperature. In this case, the nip pressure was adjusted so as to yield a finished fabric containing 3%, by weight, of chlorinated atactic polypropylene solids, as based on the dry fiber weight.

#### Example II

15 This example illustrates the preparation of fire retardant nonwoven fabrics by the process of our invention whereby the resulting fabrics contain varying amounts of chlorinated atactic polypropylene solids.

20 The basic procedure of Example I was employed to prepare nonwoven fabrics of various fiber types, including polyamide, polyacrylonitrile, rayon, and glass fibers. In all cases, the chlorinated atactic polypropylene which was utilized had a chlorine content of 15%, by weight.

| Medium for Binding Agent | Percent resin solids of medium | Percent resin solids content of resulting nonwoven fabric |
|--------------------------|--------------------------------|-----------------------------------------------------------|
| Aqueous emulsion         | 1                              | 3                                                         |
| Hexane lacquer           | 2                              | 3                                                         |
| Aqueous emulsion         | 40                             | 20                                                        |
| Hexane lacquer           | 50                             | 25                                                        |
| Aqueous emulsion         | 65                             | 280                                                       |
| Hexane lacquer           | 50                             | 280                                                       |

35 The nonwoven fabrics produced by using each of the formulations given above exhibited outstanding properties of fire retardancy and strength and were remarkably soft to the touch.

#### Example III

40 This example illustrates the vastly improved results with respect to a number of different properties in addition to fire retardancy, obtained by using chlorinated atactic polypropylene as the binding agent for nonwoven fabrics, as compared to the results obtained by using a number of conventional binding agents under the same conditions.

45 (a) The basic procedure of Example I was employed to prepare a number of viscose fiber nonwoven fabrics, each of which was bound with a different binding agent. 50 In each case, the binding agent solids constituted about 50% by weight of the resulting fabric, as based on the weight of the dry fibers. The table appearing below sets forth the binding agents used, along with certain properties exhibited by the fabrics thereby bound.

55 In determining the edge tear and percent elongation of the fabrics tested, test procedures established by the Technical Association of the Pulp and Paper Industry (TAPPI) were followed. The Finch edge tear was determined by 60 means of TAPPI test T-470-M-54, wherein higher readings indicate a proportionately stronger fabric. The percent elongation was determined by means of TAPPI test T-457-M-46.

65 The test for stiffness was carried out on an instrument called the Gurley Stiffness Tester. In using this instrument, a sample of the fabric 1 inch wide and 1.5 inches long was clamped centrally on the projected arm of the machine with the length of the sample being in a vertical position. This sample extended parallel to a freely 70 swinging pointer to which various weights were fastened. As weights were added, the arm with the clamped sample pressed against and moved the pointer, thereby giving a reading in milligrams which comprises the Gurley stiffness, wherein a higher reading indicates a proportionately stiffer and less desirable fabric.

| Binding Agent                                                        | Medium for Binding Agent | Hand           | Gurley Stiffness (mg.) | Finch Edge Tear (lb./in.) | Percent Elongation |
|----------------------------------------------------------------------|--------------------------|----------------|------------------------|---------------------------|--------------------|
| Polyvinyl acetate.....                                               | Emulsion.....            | Poor.....      | 1,400                  | 2.3                       | 18                 |
| Polyvinylidene chloride.....                                         | do.....                  | do.....        | 824                    | 4.3                       | 22                 |
| 20:80 vinyl acetate:ethyl acrylate copolymer.....                    | do.....                  | Good.....      | 444                    | 6.8                       | 44                 |
| 75:25 butadiene:acrylonitrile copolymer.....                         | do.....                  | do.....        | 380                    | 7.8                       | 55                 |
| Chlorinated atactic polypropylene (10%, by weight chlorine content). | do.....                  | Excellent..... | 230                    | 13.0                      | 84                 |

From the results represented in the above table, it can be seen that the use of chlorinated atactic polypropylene as the binding agent for nonwoven fabrics presents significant advantages over the use of any of the conventional binding agents listed above.

15

#### Example IV

The following example illustrates the actual preparation of a number of samples of chlorinated atactic polypropylene lacquers wherein each of the respective samples had a different chlorine content. These lacquers were then converted to aqueous emulsions which were used for the preparation of fire retardant nonwoven fabrics by means of the basic procedure described in Example I. It may also be noted that the various samples of chlorinated atactic polypropylene whose use was described in Examples I, II and III were all prepared by means of the process described below.

Using gaseous chlorine and sulfonyl chloride as chlorination agents, we prepared several chlorinated atactic polypropylene lacquers each of which had a resin solids content of 25%, by weight. In preparing these lacquers, the chlorination procedure described earlier in the specification was utilized. The resulting lacquers were then converted into aqueous emulsions by adding an aqueous solution of an emulsifier to the lacquer while subjecting the latter to vigorous agitation. In each case, we used 6%, of emulsifier as based on the weight of chlorinated atactic polypropylene in the respective lacquers. These emulsions, each of which had a resin solids content of 5%, by weight, were then used as binding agents for the preparation of nonwoven fabrics by means of the basic procedure described in Example I.

In the following table are presented details relating to the preparation of the various chlorinated atactic polypropylene lacquers and their subsequent conversion to aqueous emulsions.

Summarizing, this invention provides the practitioner with fire retardant nonwoven products through the use of novel binders comprising chlorinated atactic polypropylene. Variations may be made in proportions, procedures and materials without departing from the scope of the invention which is limited only by the following claims.

We claim:

1. The process of making a bonded nonwoven fabric characterized by its resistance to fire, softness and strength, said process comprising applying to a web of fibers a binding agent consisting essentially of chlorinated atactic polypropylene dispersed in a liquid medium.
2. The process of claim 1, wherein said chlorinated atactic polypropylene has a chlorine content of from about 8 to 35%, by weight.
3. The process of claim 1, wherein said binding agent is in the form of an organic solvent solution.
4. The process of claim 1, wherein said binding agent is in the form of an aqueous emulsion.
5. A bonded nonwoven fabric characterized by its fire retardancy, softness and strength, said fabric comprising a web of fibers bonded solely with a chlorinated atactic polypropylene binding agent.
6. The nonwoven fabric of claim 5, wherein said chlorinated atactic polypropylene has a chlorine content of from about 8 to 35%, by weight.
7. A bonded nonwoven fabric characterized by its fire retardancy, softness and strength, said fabric comprising a web of fibers bonded solely with the dried residue of an organic solvent solution of chlorinated atactic polypropylene.
8. A bonded nonwoven fabric characterized by its fire retardancy, softness and strength, said fabric comprising a web of fibers bonded solely with the dried residue of an aqueous emulsion of chlorinated atactic polypropylene.

| Formulation No. | Parts of Atactic Polypropylene | Catalyst Used (Parts)                       | Chlorination Agent     | Parts of Chlorinating Agent | Chlorine in Chlorinated Polymer | Emulsifying Agent     |
|-----------------|--------------------------------|---------------------------------------------|------------------------|-----------------------------|---------------------------------|-----------------------|
| 1.....          | 100                            | Lauroylperoxide (0.3).....                  | Sulfonyl chloride..... | 220                         | 35                              | Polyvinyl alcohol.    |
| 2.....          | 100                            | Ferric chloride (0.3).....                  | Chlorine.....          | 94                          | 26                              | Do.                   |
| 3.....          | 100                            | Ferric chloride and Iodine (0.3) (0.1)..... | do.....                | 60                          | 18                              | Do.                   |
| 4.....          | 100                            | Ferric chloride (0.3).....                  | do.....                | 45                          | 11                              | Oleic acidmorpholine. |
| 5.....          | 100                            | do.....                                     | do.....                | 30                          | 8                               | Polyvinyl alcohol.    |

#### References Cited by the Examiner

#### UNITED STATES PATENTS

- 3,126,297 3/1964 Diamantopoulos et al. - 117—140  
 3,192,188 6/1965 Orthner et al. ----- 260—88.2  
 3,228,791 1/1966 Armour et al. ----- 117—138.8

WILLIAM D. MARTIN, Primary Examiner.

T. G. DAVIS, Assistant Examiner.